

## UNITED STATES PATENT OFFICE.

LOUIS CHARLES DREFAHL, OF LAKewood, OHIO, ASSIGNOR TO THE GRASSELLI CHEMICAL COMPANY, OF CLEVELAND, OHIO, A CORPORATION OF OHIO.

## MANUFACTURE OF CHROMATES.

No Drawing.

Application filed March 1, 1923. Serial No. 622,206.

*To all whom it may concern:*

Be it known that I, LOUIS CHARLES DREFAHL, a citizen of the United States, residing at Lakewood, in the county of Cuyahoga and State of Ohio, have invented certain new and useful Improvements in the Manufacture of Chromates, of which the following is a specification.

This invention relates to a process for 10 the oxidation of chromium compounds and is particularly applicable to the production of chromates from chromium ores.

According to the well known and usual accepted practice for the production of 15 chromium salts, chromium oxid or finely divided chromium ore or chromium bearing material is mixed with a compound of an alkali-forming metal such as, alkali or alkaline earth metal oxid, hydroxid or carbonate or mixtures thereof, and the mixture is roasted at a suitable temperature in either a reverberatory or muffle furnace in the presence of a large excess of air. During the roasting operation the mixture is stirred 20 or rabbled either mechanically or by hand. In such processes the heat necessary to raise the constituents of the mixture to reaction temperature is derived from the burning of fuel extraneously of the mixture in a suitable fire box or combustion chamber.

According to one common method of making chromate salts from chromium ore a charge consisting of ore, soda ash and lime in suitable proportions is roasted in a hand 25 operated reverberatory furnace externally fired with coal, the charge being introduced into the furnace at a point remote from the bridge wall and advanced by hand through the furnace toward the bridge wall 30 as the oxidation progresses. About six or eight hours are required for the complete roasting of a batch of ore. The temperature at which oxidation seems to proceed favorably is in the neighborhood of 1500° F. The 35 roasted mass is then leached for the recovery of soluble chromium salts.

In this process and the other known processes referred to the presence of uncon-

sumed fuel in contact with the charge is avoided. When the process is carried out 50 in a reverberatory furnace air is introduced onto the hearth and is present at all times in considerable excess of a quantity sufficient to complete the combustion of unburned fuel coming from the fire box and an excess of air or oxygen is provided for 55 the oxidation of the chromium content of the charge to chromate. In the usual practice the presence of lime in the furnace batch is necessary in order to avoid fusing 60 of the mass whereby oxidation would be impeded. The presence of lime in the batch however results in a considerable loss of 65 chromium due to the formation of calcium chromate and other calcium-containing chromium compounds which are not readily dissolved in the dissolution process.

While carrying on development work on 70 the oxidation of chromium ores by means of known processes for the purpose of ascertaining the conditions necessary for maximum recovery of chromium salts it occurred to me that the oxidation might be successfully carried out in a very unusual manner which, for convenience, I shall call 75 blast-roasting. According to this process instead of heating the chromium-containing material by the combustion of fuel extraneously of the charge, the fuel is mixed with the chromium-containing material and the mixture is treated in a suitable apparatus such as a Huntington-Heberlein sintering pot or a Dwight-Lloyd continuous sintering apparatus. The combustion of the fuel in the charge generates sufficient heat to bring 80 the entire mass to a temperature suitable for the proper absorption of oxygen in the form of atmospheric air or oxygen applied to the mass either by suction or blast.

In applying the new process to the manufacture of chromates, I prefer to operate 85 with mixtures of chromium ore or chromium bearing material, soda ash and a suitable fuel, preferably petroleum coke or charcoal. The proportions of the constituents will 90 vary to a considerable degree depending up-

on the nature and composition of the chromium bearing material and the fuel employed. Any suitable fuel may be employed such as petroleum coke, charcoal, coke, coal, tars and oils.

Petroleum coke and charcoal are preferred because they contain very small amounts of ash producing constituents.

According to my process lime is not a necessary constituent of the charge but a charge containing lime may be satisfactorily treated.

A suitable mixture or charge may be made up as follows:

15 100 parts by weight of chromium ore (containing 50% Cr<sub>2</sub>O<sub>3</sub>).

110 parts by weight of lime (CaO).

80 parts by weight of soda ash (containing 58% Na<sub>2</sub>O equivalent).

20 67 parts by weight of fuel (charcoal or petroleum coke).

The above are mixed and dampened with sufficient water to form a mass suitable for feeding.

25 The charge is fed into suitable sintering apparatus in which the fuel of the charge is burned by a strong blast of air supplied either by suction or by blast whereby the charge is brought to a suitable temperature

30 for the oxidation of the chromium content of the charge to a higher state of oxidation with the concomitant formation of chromate salts. It is of course understood that air or oxygen is supplied in quantity sufficient to 35 burn the fuel and also supply oxygen for the oxidation of the chromium content of the charge.

The roasted or sintered charge is then leached in the usual manner for the recovery 40 of chromate salts.

In the above example the charge contains lime but this may be omitted.

The proportions of the charge will vary widely, depending not only upon the nature 45 of the constituents of the charge but also upon the size of the charge. In general the amount of fuel required for a charge is determined by the amount necessary to bring the reacting mass to a temperature at 50 which rapid oxidation will take place, such temperature being in the neighborhood of 1500° F. or higher. In applying the new process for the oxidation of chromium ores or compounds it has been found to be possible to reduce the time required for oxidation to a fraction of that required in the hand furnacing operation described above. The process can be carried out in simple apparatus occupying little space and give 55 an excellent yield and comparatively large production. The initial cost of apparatus is materially reduced and there is a material saving in maintenance, operating labor, and fuel.

60 65 This application is a continuation in part

of my application Serial No. 532,874, filed January 30, 1922.

I claim:

1. Process of oxidizing chromium compounds which comprises blast roasting a 70 mixture of the same with a carbonaceous fuel and a compound of an alkali forming metal at a temperature in the neighborhood of 1500° F.

2. Process of oxidizing chromium compounds which comprises mixing the same with a compound of an alkali forming metal and carbonaceous fuel in quantity sufficient when burned to heat the mixture to a temperature at which the chromium compounds react with oxygen, and burning said fuel in the presence of an excess of oxygen.

3. Process of oxidizing chromium compounds which comprises mixing the same with a compound of an alkali forming metal 85 and a carbonaceous fuel substantially free from ash forming constituents, and burning said fuel in the presence of an excess of oxygen.

4. Process of making chromates which 90 comprises blast-roasting a mixture of a chromium compound with a carbonaceous fuel and a compound of an alkali-forming metal.

5. Process of making chromates which 95 comprises forming a mixture of chromium ore, carbonaceous fuel and a compound of an alkali-forming metal, said fuel in quantity sufficient when burned to heat the mixture to at least 1500° F., and burning the fuel 100 in said mixture in the presence of an excess of oxygen.

6. Process of making chromates which 105 comprises forming a mixture containing chromium oxid, a compound of an alkali metal, a compound of an alkaline earth metal, and a carbonaceous fuel in quantity sufficient when burned to heat the mixture to at least 1500° F., and burning said fuel in the presence of an excess of oxygen.

7. Process of making chromates which 110 comprises forming a mixture comprising a chromium ore, an alkali metal carbonate, and a carbonaceous fuel in quantity sufficient when burned to heat the mixture to a temperature at which oxidation of the chromium content of the ore will take place, and burning said fuel in a blast of air.

8. Process of making chromates which 115 comprises forming a mixture comprising 100 parts of chromium ore, 80 parts of soda ash and 67 parts of carbonaceous fuel, and blast-roasting said mixture.

9. Process of making chromates which 120 comprises forming a mixture comprising 100 parts of chromium ore, 110 parts of lime, 80 parts of soda ash, and 67 parts of carbonaceous fuel, and blast-roasting said mixture.

10. Process of making chromates which 125

comprises forming a mixture comprising a chromium oxid ore, an alkali metal carbonate and petroleum coke and heating said mixture to at least 1500° F. in the presence 5 of free oxygen.

11. Process of making chromates which comprises heating a mixture of a chromium

compound, a compound of an alkali-forming metal and a carbonaceous fuel to oxidizing temperature solely by combustion of the 10 fuel.

In testimony whereof, I affix my signature.

LOUIS CHARLES DREFAHL.